

## UNITED STATES PATENT OFFICE

2,381,420

## HARD WAXES AND FATTY PRODUCTS DERIVED FROM CRUDE SUGAR CANE WAXES

Royal T. Balch, Washington, D. C., assignor to Claude R. Wickard, as Secretary of Agriculture of the United States of America, and his successors in office

No Drawing. Application July 25, 1942,  
Serial No. 452,370

2 Claims. (Cl. 260—428.5)

(Granted under the act of March 3, 1883, as amended April 30, 1928; 370 O. G. 757)

This application is made under the act of March 3, 1883, as amended by the act of April 30, 1928, and the invention herein described, if patented, may be manufactured and used by or for the Government of the United States of America for governmental purposes without the payment to me of any royalty thereon.

This invention relates to hard waxes and fatty products derived from crude sugar cane waxes and to the production of them.

Crude sugar cane waxes are extracted from clarification muds, or other suitable sugar cane factory waste products, by utilization of organic solvents of the waxes. The crude waxes contain many non-wax constituents or fatty portions, dependent on the variety of sugar cane from which the muds are derived, on the method by which the muds are produced in the sugar manufacturing process, and on the solvents used for extracting the crude waxes. Some of these non-wax constituents are detrimental, if the wax is to be used industrially, and must be removed.

The object of this invention is to utilize waste products of sugar cane factories. More specifically, the objects are to convert easily and simply crude sugar cane wax into hard wax products and separate fatty portions, to separate the fatty portions into separate fractions, to produce new products, and to produce products by new processes.

Preferably, the crude waxes are extracted from non-fermented materials. The clarification muds derived in the manufacture of raw sugars usually contain the higher proportions of waxes and are, therefore, the best sources from a recovery viewpoint.

It is also preferable to dry the clarification muds at the time of their production. The drying should be to a point to render the muds substantially stable in the surrounding or storage atmosphere so that they may be stored without material change. This enables operation of the extraction plant throughout the year without variation in the muds used, thus making uniformity in the final product. The degree of drying is not sharply critical, however, in reference to the extraction process. Some moisture is desirable and moisture content as high as 30 percent does not decrease the wax yield.

In the process of extracting the crude waxes

from the muds, a number of organic solvents for the waxes may be used. Toluol, commonly known as toluene, has a number of advantages and is preferred. It is preferable to extract the wax at a temperature somewhat above its melting point, since this enhances its solubility. The solvent is recovered from the extracted residue. The crude wax solution will contain an insoluble sludge of finely divided mud particles which should be filtered out. The solvent is evaporated off, but preferably not entirely to completion, and recovered, and the crude wax, obtained as a residue still containing a proportion of solvent, is allowed to solidify either in blocks or in thin sheets. These can be chipped or broken into pieces so that they may be mixed with a selective solvent in the following described process:

The chipped or broken crude wax pieces are placed in a container and covered with a charge of selective solvent (a material which is an excellent fat solvent but which is a poor wax solvent). A number of solvents have been found suitable for this purpose, including acetone, ethyl methyl ketone, ethyl ether, petroleum and certain products, such as heptane, hexane, and those rich in pentanes. Acetone and methyl ethyl ketone are preferred to the other solvents because of their higher boiling points and less volatility and because of their tolerance toward moisture which may be a contaminant of the crude wax. The container may be closed to reduce solvent losses.

The fatty portions are separated from the crude wax by a process of diffusing into the solvent, which is preferably carried out at ordinary room temperatures of from 20° to 25° C. After standing about a day, the acetone solution (solvent containing the fatty portions) is drawn off and preferably a fresh supply of acetone is added. However, in the place of fresh acetone, an acetone solution of the fatty portions resulting from an extraction of a previous batch of crude wax may be employed. This process may be repeated, the number of times depending on the thoroughness of removal of the fatty portions desired. Generally, from three to seven times is sufficient. The solvent is recovered by distillation from both the wax residue and the fatty portion solution.

The wax residue, after being freed from acetone, is melted and allowed to solidify. It is a hard and brittle wax product, ranging in color

from dark brown to dark greenish black depending on the variety of cane from which it is derived, on the methods used in the sugar manufacturing process, and on the solvents used for extracting the crude waxes. Typical analyses of hard wax products thus obtained from clarification muds from raw sugar factories are shown below:

|                       |           |
|-----------------------|-----------|
| Saponification values | 27.2-53.3 |
| Acid values           | 9.7-11.4  |
| Iodine number (Hanus) | 21.5-19.8 |

Some sterols are present but not in detrimental quantities. Waxes of these characteristics are useful for industrial purposes.

The acetone soluble fatty portion contains valuable mixed fractions which are also recovered. Such portion can be resolved without difficulty into three fractions: first, a crystalline product composed principally of sterols; second, a semi-solid product composed principally of free fatty acids; and third, a remaining residue.

The crystalline sterol fraction is recovered from a fairly concentrated solution of the fatty portion in acetone. This solution may be obtained by distilling only part of the acetone from the fatty portion solution remaining after separation of the hard wax. The concentrated solution is cooled to crystallize the sterols which are filtered off. The sterols thus obtained are purified by recrystallization to obtain a stable mixture. This fraction is a white or pale yellow crystalline mixture composed mainly of sterols. Such mixtures have been found to have melting points of 127-142° C., and specific rotation  $[\alpha_D^{20}]$  values from 32 to 44.3. Irradiation of said sterols by ultraviolet light yields a product having vitamin D potency.

After removal of the crystalline sterols, the acetone is recovered by evaporation from the remaining solution, and the free fatty acid fraction is obtained from the residue by subjecting it to an alcohol extraction. This fraction is a brown semi-solid substance composed mainly of free fatty acids mixed with some sterols and other minor constituents.

After removal of both the crystalline sterol

fraction and the free fatty acid or alcohol soluble fraction from the fatty portion, the remaining residue fraction is a dark colored mass, semi-solid at ordinary room temperatures, rich in natural oils, and other fat-like sugarcane compounds, and colored with plant pigments which are extremely soluble in fats. This fraction contains a substantial proportion of carotene or provitamin A.

It may not be practical to recover the constituents such as sterols, fatty acids, oils, or other fat-like compounds in pure forms, but the three mixed fractions above-described have commercial uses and are easily obtained.

Having thus described my invention, I claim:

1. A method of separating crude sugar cane wax into various constituents comprising mixing pieces of the crude wax with acetone and permitting the acetone to dissolve the fatty portions and not the hard wax constituents, separating the solution from the mixture and recovering the hard wax constituents, distilling off a portion of the acetone from the solution to give a fairly concentrated solution, cooling the concentrated solution to crystallize a sterol fraction therein, and separating and recovering the crystalline sterol fraction therefrom.

2. A method of separating crude sugar cane wax into various constituents comprising mixing pieces of the crude wax with acetone and permitting the acetone to dissolve the fatty portions and not the hard wax constituents, separating the solution from the mixture and recovering the hard wax constituents, distilling off a portion of the acetone from the solution to give a fairly concentrated solution, cooling the concentrated solution to crystallize a sterol fraction therein, separating and recovering the crystalline sterol fraction therefrom, evaporating the acetone from the remaining solution, subjecting the residue remaining after evaporation of the acetone to an alcohol extraction to recover a free fatty acid fraction, and recovering the residue remaining after extraction of the free fatty acid portion.

ROYAL T. BALCH.

### Certificate of Correction

Patent No. 2,381,420.

ROYAL T. BALCH

August 7, 1945.

It is hereby certified that error appears in the printed specification of the above numbered patent requiring correction as follows: Page 2, first column, lines 35 and 36, strike out "rotation  $[\alpha_D^{20}]$  values from 32 to 44.3." and insert instead rotation  $[\alpha]_D^{20}$  values of from -32 to -44.3.; and that the said Letters Patent should be read with this correction therein that the same may conform to the record of the case in the Patent Office.

Signed and sealed this 19th day of March, A. D. 1946.

[SEAL]

LESLIE FRAZER,  
First Assistant Commissioner of Patents.

from dark brown to dark greenish black depending on the variety of cane from which it is derived, on the methods used in the sugar manufacturing process, and on the solvents used for extracting the crude waxes. Typical analyses of hard wax products thus obtained from clarification muds from raw sugar factories are shown below:

|                       |           |
|-----------------------|-----------|
| Saponification values | 27.2-53.3 |
| Acid values           | 9.7-11.4  |
| Iodine number (Hanus) | 21.5-19.8 |

Some sterols are present but not in detrimental quantities. Waxes of these characteristics are useful for industrial purposes.

The acetone soluble fatty portion contains valuable mixed fractions which are also recovered. Such portion can be resolved without difficulty into three fractions: first, a crystalline product composed principally of sterols; second, a semi-solid product composed principally of free fatty acids; and third, a remaining residue.

The crystalline sterol fraction is recovered from a fairly concentrated solution of the fatty portion in acetone. This solution may be obtained by distilling only part of the acetone from the fatty portion solution remaining after separation of the hard wax. The concentrated solution is cooled to crystallize the sterols which are filtered off. The sterols thus obtained are purified by recrystallization to obtain a stable mixture. This fraction is a white or pale yellow crystalline mixture composed mainly of sterols. Such mixtures have been found to have melting points of 127-142° C., and specific rotation  $[\alpha_D^{20}]$  values from 32 to 44.3. Irradiation of said sterols by ultraviolet light yields a product having vitamin D potency.

After removal of the crystalline sterols, the acetone is recovered by evaporation from the remaining solution, and the free fatty acid fraction is obtained from the residue by subjecting it to an alcohol extraction. This fraction is a brown semi-solid substance composed mainly of free fatty acids mixed with some sterols and other minor constituents.

After removal of both the crystalline sterol

fraction and the free fatty acid or alcohol soluble fraction from the fatty portion, the remaining residue fraction is a dark colored mass, semi-solid at ordinary room temperatures, rich in natural oils, and other fat-like sugarcane compounds, and colored with plant pigments which are extremely soluble in fats. This fraction contains a substantial proportion of carotene or provitamin A.

It may not be practical to recover the constituents such as sterols, fatty acids, oils, or other fat-like compounds in pure forms, but the three mixed fractions above-described have commercial uses and are easily obtained.

Having thus described my invention, I claim:

1. A method of separating crude sugar cane wax into various constituents comprising mixing pieces of the crude wax with acetone and permitting the acetone to dissolve the fatty portions and not the hard wax constituents, separating the solution from the mixture and recovering the hard wax constituents, distilling off a portion of the acetone from the solution to give a fairly concentrated solution, cooling the concentrated solution to crystallize a sterol fraction therein, and separating and recovering the crystalline sterol fraction therefrom.

2. A method of separating crude sugar cane wax into various constituents comprising mixing pieces of the crude wax with acetone and permitting the acetone to dissolve the fatty portions and not the hard wax constituents, separating the solution from the mixture and recovering the hard wax constituents, distilling off a portion of the acetone from the solution to give a fairly concentrated solution, cooling the concentrated solution to crystallize a sterol fraction therein, separating and recovering the crystalline sterol fraction therefrom, evaporating the acetone from the remaining solution, subjecting the residue remaining after evaporation of the acetone to an alcohol extraction to recover a free fatty acid fraction, and recovering the residue remaining after extraction of the free fatty acid portion.

ROYAL T. BALCH.

#### Certificate of Correction

Patent No. 2,381,420.

ROYAL T. BALCH

August 7, 1945.

It is hereby certified that error appears in the printed specification of the above numbered patent requiring correction as follows: Page 2, first column, lines 35 and 36, strike out "rotation  $[\alpha_D^{20}]$  values from 32 to 44.3." and insert instead rotation  $[\alpha]_D^{20}$  values of from -32 to -44.3.; and that the said Letters Patent should be read with this correction therein that the same may conform to the record of the case in the Patent Office.

Signed and sealed this 19th day of March, A. D. 1946.

[SEAL]

LESLIE FRAZER,  
First Assistant Commissioner of Patents.